# EUROPEAN PATENT SPECIFICATION

(11) **EP 0 085 726 B1**
(45) Date of publication and mention of the grant of the patent: **02.04.1986**
(21) Application number: 82100846.3
(22) Date of filing: 04.02.1982
(51) Int. Cl.: B22D 17/12

(54) **Method and apparatus for vertical die casting**
Verfahren und Einrichtung für das vertikale Spritzgiessen
Procédé et appareil pour le moulage par injection verticale

(43) Date of publication of application: 17.08.1983
(73) Proprietor: TOYOTA JIDOSHA KABUSHIKI KAISHA, Aichi-ken 471 (JP)
(72) Inventor: Tokui, Masaaki, Toyota-shi Aichi-ken (JP); Masaoka, Toshika, Toyota-shi Aichi-ken (JP); Ota, Atsushi, Toyota-shi Aichi-ken (JP); Ito, Takeharu, Toyota-shi Aichi-ken (JP)
(74) Representative: Tiedtke, Harro, Dipl.-Ing.

## Description

The present invention relates to a method and an apparatus for properly charging the molten metal in a vertical die casting, according to the preamble of claim 1 or claim 4 respectively.

As is well known the die casting method has been widely employed owing to its high-precision performance among a variety of casting methods. Among them, in particular, the vertical casting method has been extensively used since it allows little amount of gas to be involved within the cast product.

A method and an apparatus for vertical die casting is described in DE-A-27 14 305, wherein a predetermined amount of molten metal is introduced into a metering chamber from which it is charged under pressure through a connecting channel into a cavity of a mold. By introducing a pressure piston into the metering chamber the molten metal is pressurized and thereby raises in the connecting channel into the mold cavity which lies at a higher level than the upper level of the metered molten metal in the metering chamber.

According to a conventionally employed general vertical die casting as shown in Figure 1, a pouring gate 9 is formed by a sleeve 5 that forms a sprue runner 4 connected to °a cavity that is defined by the upper and lower molds 1 and 2, a counter plunger 7 is urged by a counter cylinder 8 to close the gate, a molten metal 10 is supplied in the state that the gate is closed, a pressure plunger 12 is lowered by a pressure cylinder 11, and the counter plunger 7 is lowered by the counter cylinder 8, so that the molten metal 10 is charged into the cavity 3 through the sprue runner 4 which is opened. To obtain satisfactory cast products, no gas should be caught in the molten metal 10 that is charged in the cavity 3, no cold shut should exist in the molten metal, so that the product should have a high specific gravity.

In charging the molten metal 10 into the cavity 3, if the molten metal is charged only by the descending action of the counter plunger 7 while the pressure plunger 12 does not pressurize the molten metal 10 in the sleeve, cold shut will develop in the molten metal so that unsatisfactory products are obtained.

To cope with this problem, the gate 9 is closed by the counter plunger 7 in the initial stage, and the counter plunger 7 is allowed to descend after the molten metal 10 is pressurized by the pressure plunger 12. In this case, the descending rate of the pressure plunger 12 is set to be faster than that of the counter plunger 7 taking the charging rate into consideration, and the speed of the plunger 12 is set to a high value.

Therefore, the pressure is exerted on the molten metal 10 by the pressure plunger 12 before the descending counter plunger 7 passes over the gate 9, i.e., before the gate is completely opened, whereby the molten metal is injected at high speeds into the cavity 3 from the opening of the gate. Accordingly, the splashes of molten metal adhere to the interior of the cavity 3 before it is fully charged with the molten metal; this means that part of the molten metal solidifies early and does not fuse together with the subsequently charged molten metal, giving rise to the occurrence of cold shut.

Furthermore, since the charging of the molten metal does not take place uniformly, gas present in the cavity is stirred and caught by the molten metal. This fact also yields to unsatisfactory products.

In the conventional method, the casting conditions were unstable, and the defects tended to develop due to the above-mentioned causes.

Therefore, an object of the present invention is to provide a method according to the preamble of claim 1 and an apparatus according to the preamble of claim 4 for production of cast products in a vertical die casting which are free from the defect such-as gas-catching and cold shut. More specifically the object of the present invention is to provide a die casting method and an apparatus for production of cast products which is characterized by smooth and continuous casting free from the gas-catching and cold shut.

This object is achieved as regards the new method by the method steps indicated in the characterizing part of claim 1, and as regards the new die casting apparatus by the features indicated in the characterizing part of claim 4.

According to the present invention the molten metal is charged into the cavity due to its own weight at the initial stage, and then the charging of the cavity is completely effected by the pressurizing action of the pressure plunger.

These and other objects and many of the attendant advantages of this invention will be readily appreciated as the same becomes better understood by reference to the following detailed description of the preferred embodiment when considered in connection with the accompanying drawings, in which
Figure 1 is a diagram illustrating a vertical die casting according to a conventional art;
Figs, 2 and 3 are diagrams illustrating an apparatus and a manufacturing process according to the present invention.
Fig. 4 is a view illustrating the sprue runner of the embodiment in Figs. 2 and 3 on an enlarged scale; and
Fig. 5 is a diagram illustrating experimental data.

In a vertical die casting to which the present invention relates, the molten metal is supplied into a sleeve while the gate is closed, and the gate is then opened so that the molten metal is charged from the sprue runner into the cavity due to the descending motion of the pressure plunger and counter plunger. According to the present invention, the cavity is charged with the molten metal at two stages: after the molten metal is supplied into the sleeve, the molten metal at first is charged smoothly into the cavity via the runner at the initial stage through lowering a lower sleeve by a descending means, and then the cavity is completely charged with the molten metal while being pressurized by the pressurizing action of the descending pressure plunger at a specified speed.

Namely, according to the present invention, the molten metal is supplied into the sleeve while the lower sleeve, at first, is brought into contact with the upper sleeve to close the gate, the lower sleeve is allowed to descend thereby to open the gate accompanying the descending motion of the pressure plunger, a predetermined amount of molten metal is allowed to smoothly flow due to its own weight, and the pressure plunger gives pressure upon the molten metal under the condition in which the flow of molten metal is not terminated, so that the molten metal is charged into the cavity through the sprue runner, thereby to obtain a satisfactory product without splashes of molten metal, without containing gases, and without cold shut.

The present invention will be explained more in detail with reference to one embodiment shown in Figs. 2-4. In these figures, the same reference numerals represent the same as or similar to the parts in Fig. 1.

Symbol A denotes a vertical die casting apparatus which is used to produce cast products free from the defect such as gas-catching and cold shut, in which a reference numeral 3 is a cavity which is defined by an upper mold 1 and a lower mold 2, a reference numeral 13 is a core secured within the cavity 3. As shown in detail in Fig. 4, the cavity 3 is located at a position lower than the gate 9, and a sprue runner 4' is downwardly tilted at an angle between, for example, 5° to 45°, extending from the gate 9 to the cavity.

An upper sleeve 5' is secured to the upper mold 1, and a lower sleeve 5" which is vertically movable with respect to the lower mold 2 and coupled to a hydraulic cylinder 14 that works as a lowering and lifting means is brought into close contact with the lower end of the upper sleeve 5' at the gate 9 thereby to close the gate. A counter plunger 7 is slidably inserted inside the lower sleeve 5" and is connected to a counter cylinder 8 located at a lower position.

A pressure plunger 12 is fitted into the upper sleeve 5' and is coupled to a pressure cylinder 11 located at an upper position. A dog 16 provided on the rod 15 is designed to be able to come into contact with a limit switch 17 that is attached to a frame (not shown). The limit switch is connected to a hydraulic pump actuating device and the hydraulic cylinder 14, if need be via a suitable relay (not shown).

For the purpose of convenience, the ratio of sectional area of the pouring gate 9 to the volume of product (volume of the cavity) has been set to be 0.01 to 0.08 cm-'.

The hydraulic mechanism on the pressurizing side of the pressure cylinder 11 is so designed that a pressure ratio determining device (not shown) may determine the relative pressure of the pressure plunger 12 relative to the counter plunger 7.

In the vertical die casting apparatus A, the lower sleeve 5" is raised during the initial stage by the lowering and lifting means 14 to come into intimate contact with the upper sleeve 5', thereby to close the gate 9.

Under this condition, the predetermined amount of the molten metal 10 from a molten metal inlet 18 is supplied into the upper sleeve 5', and a piston of the pressure cylinder 11 is actuated to lower the pressure plunger 12.

When the dog 16 of rod 15 of the pressure plunger 12 comes into contact with the limit switch 17 located at a preset position, the lowering and lifting means 14 is operated via the relay before the pressure plunger 12 reaches the molten metal 10, whereby the lower sleeve 5" is lowered to open the gate 9.

Since the pressure plunger 12 has not yet reached the state to exert the pressure onto the molten metal, the molten metal 10, i.e. a sub-amount of metal flows by its own weight into the cavity 3 through the sprue runner 4' that is downwardly tilted at an angle a between 5° and 45°.

In this case, the molten metal 10 flows naturally through the sprue runner that is downwardly tilted. To obtain an optimum flow rate and flow capacity, however, the rate of cross sectional area of pouring gate to the volume of the product is preferably set to lie in the range from 0.02 to 0.05 cm⁻¹.

Thus, the apparatus according to the present invention is so designed that when a sub-amount of more than 10% of the molten metal to be charged into the cavity flows into the cavity by its own weight, the pressure plunger 12 comes into contact with the molten metal 10 lest the molten metal should cease to flow and the molten metal 10 is pressurized by the pressure plunger, so that it is charged into the cavity 3 through the sprue runner 4" under pressure.

Here, the above-mentioned problems seen in the conventional method arises if the molten metal gushes vigorously into the cavity. According to the present invention, therefore, the molten metal is charged under pressure at a speed which does not exceed four times speed at the gate at which the molten metal is allowed to flow by its own weight, and, preferably, does not exceed two times the speed at the initial stage.

By so constructing, the molten metal 10 is charged at a low rate into the cavity 3. Consequently, no cold shut is formed, gas is not agitated in the cavity, and no gas is captured in the molten metal, so that a die casted product is obtained satisfactorily.

Further, since the molten metal is charged at a low speed under a low pressure, the core is not damaged or bitten and even a sand core can be used.

When the charging of the molten metal is finished, the molten metal is pressurized at a predetermined pressure by the pressure plunger 12 and then, the molten metal is pressurized again by the counter plunger 7.

Finally, the mold is split to take out the product. The mold is then reset, and the molten metal is supplied again.

Fig. 5 shows the comparison results between the embodiment of the present invention and the conventional art, in which the abscissa represents the pressure P (kg/cm²) exerted on the molten metal by the pressure plunger, and the ordinate represents the specific gravity p of the die cast product. It will be understood that the product of the present invention represented by a curve C' has increased density compared with the product of the conventional art represented by a curve C, and therefore the present invention can provide a more excellent product having the compact structure.

As a matter of course, the embodiment of the present invention should not be limited to the above-mentioned example only. For instance, the core may be employed in the undercut type and the sprue runner may be curved, not straight.

The invention can also be adapted for effecting complicated profile die casting without using a core.

The charging rate and the charging capacity of the molten metal, by its own weight'i.e. the sub-amount of molten metal, the timing at which the pressure plunger comes into contact with the molten metal, the pressure to be exerted on the molten metal, and the charging rate under the. pressure can be suitably determined. Further, the means for opening and closing the gate is not limited to the lower sleeve, but the gate may be opened and closed by the counter plunger.

According to the present invention as mentioned above, the molten metal is supplied into the sleeve, i.e. a metering chamber while the gate is closed, and the gate then is opened before the pressure is exerted on the molten metal by the pressure plunger, so that a sub-amount of the molten metal is charged into the cavity as smoothly as possible by its own weight. The molten metal is charged at a slow speed without being pressurized, and does not gush into the cavity to adhere to the interior surfaces thereof followed by hardening. Thus, the molten metal is charged into the cavity in the form of laminated layer. Therefore, no cold shut is formed, gas is not stirred up in the cavity, no gas is captured by the molten metal, so that the excellent die cast product is obtained.

Then, the molten metal is charged under pressure by the pressure plunger after the predetermined amount i.e. sub-amount of the molten metal is allowed to flow into the cavity by its own weight without interruption. Therefore, the decrease of flow rate by the weight of the molten metal is compensated, and the molten metal is reliably charged at low speed; the satisfactory products can be obtained without cold shut and gas-catching.

Thus, according to the present invention, excellent products having undercuts and cavities can be obtained using a core without difficulty, and the merits of the vertical die casting method can be fully utilized.

In the casting apparatus of the present invention, as mentioned above, the lower sleeve is lowered from the upper sleeve by the lowering and lifting means so that the gate can be opened and closed, and the sprue runner which connects the gate to the cavity is so tilted that the molten metal can flow into the cavity by its own weight. Therefore, as the gate is opened by the lower sleeve, the molten metal at first freely flows into the cavity by its own weight alone, and the excellent product is obtained without cold shut or without containing gas.

## Claims

1. A vertical die casting method in which a predetermined amount of molten metal (10) is introduced into a metering chamber from which it is charged under pressure through a sprue runner (4') into a cavity (3) of a mold (1, 2), characterized in that before completely charging the molten metal (10) under pressure a predetermined sub-amount of metal is precharged while being allowed to flow exclusively under the influence of gravity forces into said cavity (3).

2. The method as claimed in claim 1, characterized in that the speed at which the charging under pressure is carried out is less than four times the speed at which the pre-charging is carried out.

3. The method as claimed in claim 1 or 2, characterized in that the speed at which the charging under pressure is carried out is less than two times the speed at which the pre-charging is carried out.

4. A vertical die casting apparatus comprising
- an upper mold (1) and a lower mold (2) defining a cavity (3) therebetween;
- a sleeve (5', 5") positioned inside of said molds (1, 2);
- a gate (9), opened and closed, in said sleeve (5',5");
- a sprue runner (4'), connecting said gate (9) and said cavity (3),
- a pressure plunger (12) which serves to pressurize molten metal (10) to be charged into said cavity (3);
means (11) for actuating said pressure plunger (12);
- a counter plunger (7); and,
- means for lowering and lifting said counter plunger (7), characterized in that
- said sleeve is formed by an upper sleeve (5') and a lower sleeve (5") which is actuated by means (14) for lowering and lifting said lower sleeve (5") and thereby opening and closing said gate (9) under the control of limit means (16, 17) which are actuated by the movement of the pressure plunger (12); and in that
- means (8) are provided for lowering and lifting said counter plunger (7) which serves to pressurize the molten metal (10) after the pressurizing by the pressure plunger (12) has been terminated.

5. The die casting apparatus as claimed in claim 4, wherein said sprue runner (4') is tilted downwardly at an angle between 5° to 45°.

6. The die casting apparatus as claimed in claims 4 or 5, characterized in that the ratio of the sectional area of said gate (9) to the volume of said cavity (3) is 0.01 to 0.08 cm-'.

7. The die casting apparatus as claimed in claim 6, characterized in that said ratio is 0.02 to 0.05 cm⁻'.

## Revendications

1. Procédé de coulée verticale sous pression dans lequel une quantité prédéterminée de métal fondu (10) est introduite dans une chambre de dosage à partir de laquelle'elle est chargée sous pression par l'intermédiaire d'un conduit de coulée (4') dans une cavité (3) d'un moule (1, 2), caractérisé en ce que, avant le chargement complet du métal fondu (10) sous pression, une quantité auxiliaire prédéterminée de métal est préchargée en la laissant s'écouler exclusivement sous l'influence des forces de gravité dans ladite cavité (3).

2. Le procédé tel que revendiqué dans la revendication 1, caractérisé en ce que la vitesse à laquelle le chargement sous pression est effectué est inférieure à quatre fois la vitesse à laquelle le préchargement est effectué.

3. Le procédé tel que revendiqué dans la revendication 1 ou 2, caractérisé en ce que la vitesse à laquelle le chargement sous pression est effectué est inférieur à deux fois la vitesse à laquelle le préchargement est effectué.

4. Une machine de coulée verticale sous pression comprenant:
- un moule supérieur (1) et un moule inférieur (2) définissant entre eux une cavité (3);
- un manchon (5', 5") positionné à l'intérieur desdits moules (1, 2);
- une porte (9), ouverte et fermée, dans ledit manchon (5', 5");
- un conduit de coulée (4') reliant ladite porte (9) à ladite cavité (3);
- un piston plongeur de pressurisation (12) qui sert à pressuriser le métal fondu (10) à charger dans ladite cavité (3);
- un moyen (11) pour actionner ledit piston plongeur de pressurisation (12);
- un contre-piston (7);
- un moyen pour faire descendre et monter ledit contre-piston (7), caractérisé en ce que:
- ledit manchon est formé par un manchon supérieur (5') et un manchon inférieur (5") qui est actionné par un moyen (14) pour faire monter et descendre ledit manchon inférieur (5") et pour assurer ainsi une ouverture et une fermeture de ladite porte (9) sous la commande de moyens de limitation (16, 17) qui sont actionnés par le mouvement du piston plongeur de pressurisation (12);
et en ce que:
- des moyens (8) sont prévus pour faire monter et descendre ledit contre-piston (7) qui sert à mettre en pression le métal fondu (10) après l'achèvement de la mise en pression par le piston plongeur de pressurisation (12).

5. La machine de coulée sous pression telle que revendiquée dans la revendication 4, dans laquelle ledit conduit de coulée (4') est incliné vers le bas d'un angle compris entre 5° et 45°.

6. La machine de coulée sous pression telle que revendiquée dans les revendications 4 ou 5, caractérisée en ce que le rapport entre la section de ladite porte (9) et le volume de ladite cavité (3) est compris entre 0,01 et 0,08 cm-^{1.}

7. La machine de coulée sous pression telle que revendiquée dans la revendication 6, caractérisée en ce que ledit rapport est compris entre 0,02 et 0,05 cm-¹.

## Patentansprüche

1. Vertikalspritzgießverfahren, bei dem eine vorgegebene Menge flüssigen Metalls (10) in eine Bemessungskammer eingeführt wird, ausder es unter Druck durch einen Einguß (4') in eine Matrize (3) einer Preßform (1, 2) geladen wird, dadurch gekennzeichnet, daß vor der Vollbeladung durch flüssiges Metall (10) unter Druck eine vorgegebene Teilmenge Eisen vorgeladen wird, wobei das Eisen ausschließlich unter Schwerkrafteinfluß in die Matrize (3) fließen kann.

2. Verfahren nach Anspruch 1, dadurch gekennzeichnet, daß die Geschwindigkeit, mit der die Druckbeladung durchgeführt wird, weniger als viermal so groß wie die Geschwindigkeit ist, mit der die Vorbeladung durchgeführt wird.

3. Verfahren nach Anspruch 1 oder 2, dadurch gekennzeichnet, daß die Geschwindigkeit, mit der die Druckbetadung.durchgeführt wird, kleiner als zweimal so groß wie die Geschwindigkeit ist, mit der die Vorbeladung durchgeführt wird.

4. Vertikalspritzgießvorrichtung mit einem oberen Formteil (1) und einem unteren Formteil (2), die zwischen sich eine Matrize ausbilden, einem Zylinder (5', 5"), der innerhalb der beiden Formteile (1, 2) angeordnet ist, einer Öffnung (9), die in dem Zylinder (5', 5") geöffnet und geschlossen wird, einem Einguß (4'), der die Öffnung (9) und die Matrize (3) miteinander verbindet, einem Druckkolben (12), der zur Druckbeaufschlagung des flüssigen Metalls (10) dient, das in die Matrize (3) geladen werden soll, einer Betätigungseinrichtung (11) für den Druckkolben (12), einem Gegenkolben (7) und einer Heb- und Senkvorrichtung für den Gegenkolben (7), dadurch gekennzeichnet, daß der Zylinder durch einen oberen Zylinder (5') und einen unteren Zylinder (5") gebildet wird, wobei der untere Zylinder (5") durch eine Heb-und Senkvorrichtung (14) für den unteren Zylinder (5") betätigt wird und dadurch gesteuert von Begrenzungsmitteln (16, 17), die durch die Bewegung des Druckkolbens (12) betätigt werden, die Öffnung (9) öffnet und schließt, und daß eine Heb- und Senkvorrichtung (8) für den Gegenkolben (7) vorgesehen ist, die dazu dient, das flüssige Metall (10) mit Druck zu beaufschlagen, nachdem die Druckbeaufschlagung durch den Druckkolben (12) beendet ist.

5. Vorrichtung nach Anspruch 4, bei der der Einguß (4') in einem Winkel zwischen 5° und 45° nach unten geneigt ist.

6. Vorrichtung nach Anspruch 4 oder 5, dadurch gekennzeichnet, daß das Verhältnis der Teilfläche der Öffnung (9) zum Volumen der Matrize (3) zwischen 0,01 und 0,08 cm⁻¹ liegt.

7. Vorrichtung nach Anspruch 6, dadurch gekennzeichnet, daß das Verhältnis zwischen 0,02 und 0,05 cm⁻¹ liegt.
